

# UNITED STATES PATENT OFFICE.

NATHAN SULZBERGER, OF NEW YORK, N. Y.

## PROCESS OF DESENSITIZING PHOTO-SENSITIVE SILVER COMPOUNDS.

1,361,352.

Specification of Letters Patent.

Patented Dec. 7, 1920.

No Drawing. Application filed December 10, 1914. Serial No. 876,495. Renewed September 7, 1920. Serial No. 408,776.

*To all whom it may concern:*

Be it known that I, NATHAN SULZBERGER, a citizen of the United States, resident of New York city, in the county and State of New York, have invented new and useful Improvements in Processes of Desensitizing Photo-Sensitive Silver Compounds and Products Produced Thereby, of which the following is a specification.

This invention relates to improvements in the desensitizing of photo-sensitive silver compounds of films, plates, prints, and like photographic reproductions, and to the improved products produced thereby or resulting therefrom.

The invention is based upon the discovery that photo-sensitive silver compounds commonly used in photography, particularly silver chlorids, can be made fast toward the action of light or more or less completely desensitized toward light, by treating them with a suitable desensitizing solution containing therein a compound of a metal of the platinum group having a desensitizing action upon such silver compounds.

As the result of the treatment to which the negatives, prints, films and the like, containing the photo-sensitive silver compounds, are subjected, they are prevented from fading as they would otherwise do under the action of light, and they are given an improved and characteristic composition well adapting them for purposes and uses, when photographic reproduction is desired.

As an example illustrative of the process of the present invention, and the production of the improved product of the invention, the following more detailed description may be given:

A print on photographic paper, which contains such light-sensitive silver salts as silver chlorid, and which is used for copying negatives in daylight, is treated with a very weak solution of a palladium compound having a desensitizing action upon the sensitive silver compound or compounds present.

A solution of readily soluble palladium-ammonium-proto-chlorid dissolved in water is well adapted for the desensitizing solution. The bringing of the print into contact with the palladium solution results in the desensitizing of the silver compounds so that they are "fixed" against the action of light. If a part only of the print is sub-

jected to the palladium solution, and then the whole print, including both the treated and untreated parts, are exposed to the action of light, all those parts of the print which have not been treated with the palladium solution will soon become dark and be destroyed for useful photographic purposes.

The treatment of the print or like photographic reproduction with the desensitizing solution makes it unnecessary, accordingly, to subject the same to an after-treatment with a solvent for removing the silver chlorid, something which has heretofore been considered unavoidable because of the highly sensitive character toward light of the silver chlorid.

This "fixing" of the print or the like may be accomplished in cases with a solution containing as little as even one part of palladium-ammonium-proto-chlorid in five hundred parts of water.

The desensitizing process of the present invention not only desensitizes the photo-sensitive silver compounds but in certain cases, as when using daylight copying paper, very markedly brightens up the print and especially those parts of the print which have by over-exposure to light during the printing process, become objectionably dark. Such over-exposed prints or portions of prints can frequently be saved by the lightening or brightening thereof resulting from the treatment according to the present invention; so that from one viewpoint, the process of the present invention may be considered as involving both a desensitizing of the silver compounds and a brightening of dark over-exposed prints containing silver compounds.

Another advantage of the present invention is that it avoids the necessity of using and therefore of removing all traces of sodium thiosulfate, which has almost exclusively been used heretofore as a solvent for the still-sensitive silver salts of the print; so that the present process enables the saving of considerable time and of large amounts of water commonly heretofore required.

From the above description it will be seen that the desensitizing treatment is one applied directly to the prints or other photographic reproductions containing the light-sensitive silver compounds, and that this

treatment involves a simple treatment with a suitable solution containing a compound of a metal of the platinum group which is adapted for the desired desensitizing of the 5 silver compounds. Instead of the particular palladium compound above referred to, other compounds of metals of the platinum group having similar desensitizing properties, may be similarly employed. Modifications 10 in the specific procedure above described, such as will suggest themselves to those skilled in the art, are to be considered as coming within the scope of the invention and of the appended claims. Accordingly, 15 mixtures of the metal compounds belonging to the platinum group and having the desired desensitizing properties, may be employed.

The term "platinum group" includes: 20 platinum, iridium, osmium, palladium, ruthenium and rhodium.

In referring to "divalent" metal of the platinum group, and to compounds of such metal, the term "divalent" is intended to include 25 not only desensitizing divalent soluble compounds of a metal or of metals belonging to the platinum group, but also mixtures containing the same which are efficient in desensitizing toward the action of light a 30 photographic reproduction such as a photo print on paper (a positive) or the developed print on a plate or film (a negative). I include also such mixtures of compounds of metals of the platinum group which will reduce 35 a higher valency of the metal or metals of this group to the divalent form, and which are similarly efficient in the desired desensitizing action.

The claims are intended also to include 40 mixtures of the soluble desensitizing compounds of a metal or metals belonging to the platinum group with other substances which do not destroy or interfere with the desired desensitizing action of the compound or compounds of the platinum metal or metals employed.

I claim:

1. The process of desensitizing toward the 45 action of light, photo prints, films and like 50 photographic reproductions containing light

sensitive silver compounds, which comprises treating the same with a solution of palladium-ammonium-proto-chlorid.

2. The method of desensitizing photo prints, films, and like photographic reproductions containing light-sensitive silver chlorid, which comprises subjecting the same to treatment with a solution of palladium, ammonium-proto-chlorid. 55

3. A desensitized photographic reproduction containing silver compounds, said reproduction having the silver compounds thereof desensitized by treatment with a desensitizing compound of a metal of the platinum group, the said photographic reproduction containing in addition to silver constituents which have been reduced by the action of light, also silver constituents which have not been reduced by the action of light but which have been desensitized. 60

4. A desensitized photographic reproduction containing silver compounds, said reproduction having the silver compounds thereof desensitized by treatment with palladium-ammonium-proto-chlorid, said photographic reproduction containing in addition to silver constituents which have been reduced by the action of light, also silver constituents which have not been reduced by the action of light but which have been desensitized. 70

5. A desensitized photographic reproduction containing silver chlorid, which has been desensitized by treatment with a desensitizing compound of a metal of the platinum 75 group, and still containing silver compounds soluble in sodium thio-sulfate. 80

6. A desensitized photographic reproduction on a sensitized medium containing silver compounds, said reproduction containing, in addition to silver constituents which have been reduced by the action of light, also silver constituents originally sensitive and which have not been so reduced but have been desensitized without dissolution. 90

NATHAN SULZBERGER.

Witnesses:

CHARLES FISCHER,  
ALBERT O. STOCKER.